

# United States Patent

Fuchs et al.

[15] 3,639,220

[45] Feb. 1, 1972

[54] ELECTRODEPOSITION OF NICKEL

[72] Inventors: Charles F. Fuchs, Evanston, Ill.; Henry Brown, Huntington Woods, Mich.

[73] Assignee: Udylite Corporation, Warren, Mich.

[22] Filed: July 27, 1970

[21] Appl. No.: 58,700

[52] U.S. Cl..... 204/49

[51] Int. Cl..... C23b 5/08, C23b 5/46

[58] Field of Search .. 204/49, 44, 43, 112;  
117/130 E; 106/1

[56] References Cited

UNITED STATES PATENTS

2,678,910 5/1954 Brown ..... 204/49

|           |        |                  |          |
|-----------|--------|------------------|----------|
| 2,800,440 | 7/1957 | Brown .....      | 204/49   |
| 2,841,602 | 7/1958 | Brown et al..... | 204/49 X |
| 3,306,831 | 2/1967 | Cope .....       | 204/43   |
| 3,428,536 | 2/1969 | Towle et al..... | 204/49   |

Primary Examiner—G. L. Kaplan

Attorney—Stanley H. Lieberstein and William J. Schramm

[57]

## ABSTRACT

It has been found that certain unsaturated aliphatic sulfonic acids characterized by having four aliphatic carbon atoms and two separate aliphatic unsaturated linkages, such as the allene sulfonic acid  $\text{CH}_2=\text{C}=\text{C}-\text{CH}_2\text{SO}_3\text{H}$  are excellent when used in acidic nickel plating baths in making it possible to obtain lustrous ductile nickel plate over a very wide plating range. These sulfonic acids do not have critical upper concentration limits.

16 Claims, No Drawings

## ELECTRODEPOSITION OF NICKEL

This invention relates to the electrodeposition of fine-grained lustrous nickel plate from aqueous acidic nickel-plating baths. More particularly it relates to the use in nickel-plating baths of certain unsaturated aliphatic sulfonic acids characterized by having four aliphatic carbon atoms and two separate aliphatic unsaturated linkages, for the purpose of obtaining lustrous ductile plate.

14.  $\text{HC}\equiv\text{C}-\text{C}=\text{CH}-\text{SO}_3\text{H}$ 

0.05-8



TABLE II

TABLE I

|                                                                       | Conc.<br>g./l. | Conc.<br>g./l. |
|-----------------------------------------------------------------------|----------------|----------------|
| 1. $\text{CH}_2=\text{C}=\text{CH}-\text{CH}_2-\text{SO}_3\text{H}$   | 0.1-10         | 15             |
| 2. $\text{CH}_2=\text{CH}-\text{CH}=\text{CH}-\text{SO}_3\text{H}$    | 0.1-10         |                |
| 3.                                                                    | 0.05-8         | 20             |
| 4. $\text{CH}_2=\text{C}=\text{C}-\text{CH}_2-\text{SO}_3\text{H}$    | 0.05-8         |                |
| 5.                                                                    | 0.05-8         |                |
| 6. $\text{CH}_2=\text{CH}-\text{C}=\text{CH}-\text{SO}_3\text{H}$     | 0.05-8         |                |
| 7.                                                                    | 0.05-8         | 40             |
| 8. $\text{CH}_2=\text{CH}-\text{CH}=\text{C}-\text{SO}_3\text{H}$     | 0.05-8         |                |
| 9.                                                                    | 0.05-8         |                |
| 10. $\text{CH}=\text{CH}-\text{SO}_3\text{H}$                         | 0.05-8         | 55             |
| 11.                                                                   | 0.05-8         |                |
| 12. $\text{CH}=\text{CH}-\text{SO}_3\text{H}$                         | 0.05-8         |                |
| 13. $\text{HC}\equiv\text{C}-\text{CH}=\text{CH}-\text{SO}_3\text{H}$ | 0.05-8         | 75             |

It has now been found that the unsaturated aliphatic sulfonic acids shown in table I are unusually effective in decreasing the grain size and increasing the luster and brightness of nickel deposited from aqueous acidic nickel-plating baths, without seriously decreasing the ductility of the plate or the current density range of the nickel bath. The compounds of table I are more effective than the aliphatic (four) carbon atom compound: 2-butyne-1,4-disulfonic acid in that they produce brightness and luster with much lower concentrations of material, and are vastly superior to the aliphatic (four) carbon atom compound: 2-butene-1,4-disulfonic acid in producing brightness and luster at any concentration. The compounds of table I are also far superior to 2-butene-1-sulfonic acid



in producing luster without seriously decreasing the ductility of the plate or causing tensile stresses. The unsaturated aliphatic sulfonic acids of this invention cooperate to give nickel plate of high brilliance and leveling when used in conjunction with unsaturated compounds, such as those carrying the  $\text{C}=\text{N}$  unsaturated linkage, for example, pyridine, quinoline, isoquinoline and their salts and especially their quaternary salts, or the unsaturated  $\text{C}=\text{C}$  linkage as in coumarin, or the unsaturated  $\text{C}\equiv\text{C}$  linkage as in dimethylethynyl carbinol or butyne diol, or the unsaturated allene linkage as in  $\text{CH}_2=\text{C}=\text{CH}-\text{CH}_2\text{OH}$ ,  $\text{CH}_2=\text{C}=\text{CH}-\text{CH}_2\text{OC}_2\text{H}_4\text{OH}$ , and  $\text{CH}_2=\text{C}=\text{CH}-\text{CH}_2\text{OCH}_2\text{CHOHCH}_2\text{Cl}$ , or the unsaturated  $\text{C}=\text{N}$  linkage as in ethylene cyanohydrin, or the unsaturated  $\text{C}=\text{O}$  linkage as in bromal, or of combinations of these types of unsaturated compounds. When one or more of the compounds of table I are used with the above types of unsaturated compounds and with one or more of the well-known benzene and naphthalene sulfonic acids, sulfonamides and sulfonimides illustrated in table II, maximum ductility is obtained for the brilliant high levelling nickel plate.

The unsaturated aliphatic sulfonic acids illustrated in table I are effective not only in the Watts high nickel sulfate concentration baths, but also in high chloride, sulfamate or fluoroborate nickel baths or mixtures of these baths and salts. The concentrations of table I compounds in the nickel baths are not critical; though in general, no further improvements in luster or ductility are obtained with concentrations above about 10 grams per liter. The bath-soluble salts of the sulfonic acids of this invention are preferred for easier handling especially the sodium or potassium salts. In the acidic nickel baths, the compounds of table I are, of course, present mainly as the sulfonic acids and their nickel salts even if added to the baths as sodium or potassium salts or for that matter, cobalt, magnesium or other salts.

The compounds of table I may have halogen atoms substituted for some of the hydrogen atoms, with at the most two halogen atoms per molecule. The halogen atoms may be on the benzene rings as well as on the aliphatic portion of the molecules. In compound 1 of table I, for example, a chlorine or bromine atom could replace one or both of the hydrogen atoms on the carbon next to the sulfonic group with improved results in luster of the nickel plate. Also one or two fluorine, chlorine, bromine or iodine atoms can be present, for example, on the benzene ring of compound 5 of table I with slightly improved results in luster of the nickel deposit. In most cases, the improvements are only slight from the presence of halogen atoms in the compounds of table I. The best pH range for the acidic nickel-plating baths employing the compounds of table I is from about 2.5 to 5.5. The bath temperatures may be from room temperature to at least 180° F., and in this respect, the brighteners of table I used by themselves or with unsaturated compounds, such as a quaternary of pyridine or quinoline, or in conjunction with butynediol or a mono- or di-ethylene oxide adduct of butynediol are superior to the well-known brighteners of table II used alone or with the unsaturated compounds. The compound of table II may be used in amounts of from 0.1 g./l. to saturation.

Below are listed some preferred examples of baths for the production of brilliant nickel plate, with bright plate range from the highest current densities down to the very lowest current densities.

#### EXAMPLE I

|                                           | Grams per Liter |
|-------------------------------------------|-----------------|
| $\text{NiSO}_4 \cdot \text{H}_2\text{O}$  | 200-300         |
| $\text{NiCl}_2 \cdot 6\text{H}_2\text{O}$ | 30-60           |
| $\text{H}_3\text{BO}_3$                   | 40              |
| Compound 2 of table I                     | 1-4             |
| Allyl quinaldinium bromide                | 0.003-0.01      |

#### EXAMPLE II

|                                                                                                                | Grams per Liter |
|----------------------------------------------------------------------------------------------------------------|-----------------|
| $\text{NiCl}_2 \cdot 6\text{H}_2\text{O}$                                                                      | 100-220         |
| $\text{NiSO}_4 \cdot 6\text{H}_2\text{O}$                                                                      | 0-50            |
| $\text{H}_3\text{BO}_3$                                                                                        | 40              |
| Compound 1 of Table I                                                                                          | 2-4             |
| Compound 1 of Table II                                                                                         | 1-6             |
| Compound 2 of Table II                                                                                         | 1-2             |
| $\text{HOH}_2\text{C}-\text{C}\equiv\text{C}-\text{CH}_2\text{OCH}_2\text{CH}-\text{CH}_2\text{SO}_3\text{Na}$ | 0.1-0.6         |

#### EXAMPLE III

|                                           |         |
|-------------------------------------------|---------|
| $\text{NiSO}_4 \cdot \text{H}_2\text{O}$  | 150-200 |
| $\text{NiCl}_2 \cdot 6\text{H}_2\text{O}$ | 30-150  |
| $\text{H}_3\text{BO}_3$                   | 40      |
| Compound 5 of table I                     | 0.5-3   |
| Compound 1 of table II                    | 1-3     |
| Compound 8 of table II                    | 1-2     |

The plate from nickel baths with one or more of the compounds of table I present are remarkably free from pitting especially when the concentration of the compounds is about 0.5 g./l. and higher. In general, however, a surface-active agent such as sodium n-octyl sulfate or sodium 2-ethyl hexyl sulfate in concentrations of 0.1 to 1 g./l. is preferred to be used in air-agitated baths, and sodium lauryl sulfate or sodium lauryl ethoxy sulfate with non-air-agitated baths. The plate of highest brilliance as previously mentioned is obtained by the conjunctive use of unsaturated class II nickel brighteners as

shown in examples I and II.

The table I unsaturated aliphatic sulfonic acids of this invention can be used in very high concentrations in the acidic nickel-plating baths, in fact, up to saturation concentrations, which for some of the compounds, for example, compounds 1 and 2, are over 100 grams/liter. However, no further improvement of luster is obtained in concentrations above about 10 grams/liter, but since the compounds are noncritical in concentration, any concentration up to saturation concentrations can be used, preferably 0.05 to about 100 g./l.

10 The compounds of table I are just as effective as brighteners in nickel-cobalt, nickel-iron and nickel-cobalt-iron alloy plating baths. The cobalt may be as high as at least 50 percent in the plate and the iron as high as at least 40 percent, and the total of cobalt plus iron may be as high as 50 percent of the plate. With cobalt concentrations in the plate higher than about 50 percent, it is preferred to have compound 1 of table II also present in the baths. Thus, with the nickel baths and nickel plate described in this invention as in examples I, II and III, cobalt and iron may also be present in the plate to the extent of about 50 percent of the plate as combined material, or as about 50 percent of either cobalt or iron separately, and still obtain bright plate that behaves essentially like bright nickel plate. It is therefore to be understood that the claimed 15 nickel baths cover these nickel alloy plates.

20 Compounds of table I produce lustrous nickel plate even when the bath temperatures are as high as 180° to 190° F.

25 What is claimed is:

1. A bath for the electrodeposition of fine-grained lustrous 30 nickel comprising essentially an aqueous acidic nickel-plating bath containing dissolved therein at least one of the unsaturated sulfonic acids listed in table I in a concentration of about 0.05 to about 100 grams/liter.

2. A bath as claimed in claim 1 wherein there is also present 35 dissolved in said bath at least one of the compounds listed in table II in a concentration of about 0.1 gram/liter to saturation.

3. A bath as claimed in claim 2 wherein the unsaturated sulfonic acid is compound 2 of table I.

40 4. A bath as claimed in claim 2 wherein the unsaturated sulfonic acid is compound 1 of table I.

5. A bath as claimed in claim 2 wherein the unsaturated sulfonic acid is compound 5 of table I.

45 6. A bath as claimed in claim 1 wherein the unsaturated sulfonic acid is compound 2 of table I.

7. A bath as claimed in claim 1 wherein the unsaturated sulfonic acid is compound 1 of table I.

8. A bath as claimed in claim 1 wherein the unsaturated sulfonic acid is compound 5 of table I.

9. A method for electrodepositing fine-grained lustrous nickel comprising the step of electrodepositing fine-grained lustrous nickel from an aqueous acidic nickel-plating bath containing dissolved therein at least one of the unsaturated sulfonic acids listed in table I in a concentration of about 0.05 to about 100 grams/liter.

55 10. A method as claimed in claim 9 wherein there is also present dissolved in said bath at least one of the compounds listed in table II in a concentration of about 0.1 gram/liter to saturation.

60 11. A method as claimed in claim 10 wherein the unsaturated sulfonic acid is compound 2 of table I.

12. A method as claimed in claim 10 wherein the unsaturated sulfonic acid is compound 1 of table I.

65 13. A method as claimed in claim 10 wherein the unsaturated sulfonic acid is compound 5 of table I.

14. A method as claimed in claim 9 wherein the unsaturated sulfonic acid is compound 2 of table I.

15. A method as claimed in claim 9 wherein the unsaturated sulfonic acid is compound 1 of table I.

70 16. A method as claimed in claim 9 wherein the unsaturated sulfonic acid is compound 5 of table I.

\* \* \* \* \*